

## UNITED STATES PATENT OFFICE

2,593,839

## DIAZOTYPE PHOTOPRINTING MATERIAL

Saul R. Buc, Northampton County, Pa., assignor  
to General Aniline & Film Corporation, New  
York, N. Y., a corporation of Delaware

No Drawing. Application November 23, 1948,  
Serial No. 61,727

7 Claims. (Cl. 95—6)

1

This invention relates to diazotype photoprinting material and process for the manufacture thereof. More particularly, this invention relates to diazotype photoprinting material having a two-component diazotype light sensitive layer and a method for making the same.

Two-component diazotype light sensitive layers contain a light sensitive diazo compound, suitably stabilized against premature coupling prior to development of the material, together with an azo coupling component. Upon exposure of such a layer to light of locally varied intensity in accordance with an original pattern or design to be reproduced, the diazo compound is partly or completely destroyed in the light exposed portions, so that upon subjecting the layer to developing treatment as by exposure to alkaline vapors, e. g. ammonia, or treatment with an alkaline solution, the residual diazo compound couples with the azo component to form an azo dye image of the original pattern. The development is conveniently carried out in the dry process by exposing the layer to ammonia or a volatile amine, or by the wet or semi-wet process in which an alkaline developer solution is applied to the layer after exposure thereof.

To manufacture two-component diazotype layers, the sensitizing components are generally applied or deposited successively or in combination on a support such as paper, plastic materials, metals, glass or the like. For absorbent materials like paper, the sensitizing composition can be used in aqueous solution, while for plastics it has been suggested to use a solution containing an organic solvent which has a solvent or swelling action upon the plastic support.

Many of the sensitizing materials heretofore employed in two-component layers were defective in that the image lacked fastness to water and aqueous solutions because of the solubility in water of the resulting azo dye. Moreover, when incorporated in a plastic carrier, the azo dye produced on development was subject to migration or offsetting in the layer. Both of these conditions cause blurring of the image, rendering such compositions unsuitable for prints in which sharpness of the image is required.

At the same time it is desirable to use sensitizing components in diazotype layers which yield dark shades adapted to reproduce the opaque parts of the original, while at the same time having a sufficiently moderate gradation to reproduce a wide range of densities as are generally found in photographs.

Diazotype images produced with two-component layers containing resorcinol as a coupler are subject to disadvantages. When such images are formed on a plastic base, the image is sub-

2

ject to migration or offsetting, causing blurring or spreading of the lines and margins of the image. The colorations produced are not fast to washing and hence often yield a blurred image when the development is carried out by the wet or semi-wet process. The brown colorations ordinarily obtained with resorcinol have a definite reddish tint which is not desirable, especially in photographic reproductions.

10 It is an object of this invention to provide novel two-component diazotype layers which yield dark purplish-brown images having a wide range of gradation suitable for the reproduction of photographic originals, which are not subject to offsetting or migration when produced on plastic carriers, and having good fastness to water and aqueous solutions.

I have discovered that diazotype layers containing, as the azo coupling component, a 20 crystalline tetrameric condensation product of a m-polyhydric phenol (resorcinol, phloroglucinol) with an equimolecular amount of an aldehyde having the formula RCHO, wherein R is a hydrocarbon radical of 1-6 carbon atoms, yield prints 25 having dark purplish brown images of good fastness to light which do not offset or migrate in a plastic carrier and which have excellent fastness to water and aqueous solutions.

The azo coupling components employed in accordance with this invention can be conveniently 30 prepared, by the procedure of Niederl et al. in J. A. C. S. 62 (1940), pp. 2512-2513, by mixing 1 mol of resorcinol or phloroglucinol with 0.9-1 mol of a hydrocarbon aldehyde, wherein the hydrocarbon contains 1-6 carbon atoms, in aqueous or 35 aqueous alcoholic sulfuric acid of 5-10% concentration, and allowing the reaction mixture to stand without external heating until the crystalline condensation product separates. For lower aldehydes, water can be used, while for aldehydes 40 containing 4 or more carbon atoms, equal parts by weight of ethyl alcohol and water are employed as a reaction medium to retain the aldehyde solution. The concentration of the aldehyde and m-polyhydric phenol in the reaction mixture is generally 2-7%, the reaction being carried out by dissolving the m-polyhydric phenol in a portion of aqueous or aqueous alcoholic sulfuric acid, dissolving the aldehyde in the remainder of the reaction medium, and 45 gradually adding the aldehyde solution to the m-polyhydric phenol solution. The crystalline condensation product which separates from the reaction mixture on standing can be recrystallized from alcohol. The products thus obtained 50 are tetramers containing four polyhydric phenol radicals and four aldehyde radicals, together with water of crystallization. The structure of the crystalline condensation products obtained 55

from resorcinol, as given by Niederl et al., is as follows:



R being the hydrocarbon radical of the aldehyde. However, it is believed the structure may be of the open-chain type as follows:



R having the same significance as above. Corresponding derivatives of phloroglucinol have an additional hydroxyl group in the benzene rings in m-position to the other hydroxyl groups.

In preparing diazotype phototyping material containing the crystalline tetrameric condensation products described above, the latter may be applied simultaneously or successively with a light sensitive diazo compound, suitably stabilized against premature coupling, to a base or support. The products are applied in solvents adapted for impregnation of the carrier. Thus, alcohols (ethanol, methanol, isopropanol) are suitable as solvents for applying the coupling components to paper and other absorbent carriers. When plastic materials such as a cellulose ester or ether, e. g. cellulose acetate or ether cellulose, or a resinous polymer, such as polyvinyl alcohol or other polyvinyl resins, are employed as carriers, a solvent mixture is preferably employed for applying the coupling components, said mixture having a swelling or slight solvent action on the plastic carrier employed. For example, solutions containing  $\gamma$ -valerolactone in aqueous alcoholic medium (containing for example, methanol, ethanol, isopropanol and butanol) can be advantageously used for impregnating cellulose acetate.

Since the coupling components of this invention are water-insoluble or of low solubility in water, an alcoholic solution thereof can be first applied to an absorbent base such as paper, and the light sensitive diazo component, together with stabilizers, anti-oxidants and the like, subsequently applied in aqueous solution to the same base after evaporating the alcoholic solution. When a mixed solvent is employed, adapted to dissolve both the coupling component and the light sensitive diazo compound, such a solution can be used to sensitize a base in a single operation.

The light sensitive diazo compounds are preferably diazotized diamines of the benzene series, particularly those having at least one substituent on one of the amino groups. Diazotized o-amino-naphthols are also adapted for use at light sensitive diazo compounds in the two-component layers of the invention.

Additional ingredients for stabilizing the diazo

compounds against premature coupling and decomposition comprise organic acids such as formic, citric, tartaric, mellitic, and sulfosalicylic acids; anti-oxidants such as thiourea, and stabilizing salts such as zinc chloride or other halides forming complex addition products with the diazo salts, e. g. boron trifluoride. Colloidal wetting agents such as saponine are likewise advantageously included.

10 My invention will be more fully understood from the following examples wherein the parts are by weight unless otherwise indicated.

*Example 1*

15 4 grams of tetrameric crystalline condensation product of equimolecular amounts of acetaldehyde and resorcinol were dissolved in 100 cc. of ethyl alcohol, and the resulting solution coated

30 on paper. After drying, the paper was coated with a solution of the following composition:

1 cc. isopropanol  
5 cc. ethylene glycol  
5 g. citric acid  
35 5 g. zinc chloride  
5 g. thiourea  
0.1 g. saponine  
3 g. p-diethylaminobenzene diazonium chloride  
ZnCl<sub>2</sub> double salt

40 diluted with water to a volume of 100 cc.

After drying, the resulting sensitized material was exposed under an original pattern to be reproduced, such as an opaque line drawing on a translucent background or a photographic dia-positive, and thereafter developed by exposure to ammonia. A sharp purplish-brown image was obtained of excellent fastness to light, of deeper shade, and better fastness to washing than an image produced with a sensitizing composition similar to that described herein but containing resorcinol instead of the acetaldehyde resorcinol condensation product.

*Example 2*

45 A sensitizing solution was prepared having the following composition:

50 parts water  
20 parts isopropyl alcohol  
1 part zinc chloride  
60 2 parts thiourea  
10 parts  $\gamma$ -valerolactone  
5 parts sulfosalicylic acid  
5 parts formic acid  
5 parts butanol  
65 4 parts p-diethylamino-2-methyl benzene diazonium chloride ZnCl<sub>2</sub> double salt; and  
6 parts of the resorcinol acetaldehyde tetrameric condensation product of Example 1.

The resulting solution was heated to about 50° C. 70 and coated at this temperature on cellulose acetate foil and on plastic coated paper. The moderately elevated temperature was employed to maintain all of the components of the sensitizing mixture in solution. After drying, copies were made by the procedure described in Example 1.

Development can be effected either with ammonia or with an aqueous alkaline solution such as aqueous ammonia, sodium carbonate, tri-sodium phosphate, or tri-ethanolamine.

The resulting image was likewise of dark purplish-brown color, of excellent sharpness showing no migration or offsetting and of excellent fastness to light. A print obtained with diazotype material prepared in the same manner as described in this example but using resorcinol instead of the acetaldehyde resorcinol condensation product, showed substantial migration and offsetting and had a much lighter color.

Instead of the resorcinol acetaldehyde condensation product of the foregoing examples, there can be employed the corresponding crystalline tetrameric equimolecular condensation product of acetaldehyde with pholoroglucinol, or of propionaldehyde, butyraldehyde, isobutyraldehyde, hexaldehyde, or benzaldehyde with either resorcinol or pholoroglucinol, whereby images having similarly advantageous properties are obtained.

Instead of the light sensitive diazo compounds disclosed in the examples, there can be used the diazo compounds of p-ethylamino m-toluidene, p - amino - N - diethyl m-toluidene, p-amino-N-methylaniline, p-amino 2-methoxy-N-cyclohexylaniline, p-amino - N - 2' - hydroxyethylaniline, p-amino - N - ethyl-N-2'-hydroxyethylaniline, 3-aminocarbazole, 1,2-, 2,1-, or 1,4-aminonaphthol, 1,2-aminonaphthol-4-sulfonic acid, or 2,1-aminonaphthol-3,6-disulfo acid. These diazo compounds can be employed in the form of their diazonium chloride zinc chloride double salts or the corresponding boron trifluoride complex addition products.

As disclosed in the examples, alcohols such as methanol, ethanol, isopropanol and butanol can be employed as media for impregnating absorbent bases with the aldehyde polyhydric phenol condensation products of this invention, particularly when applied separately from the light sensitive diazo component, and mixed solvents containing water, alcohols and a softening agent for plastics such as  $\gamma$ -valerolactone, can be used as a medium for applying the light sensitive diazo component as well as coupling components of this invention in a single operation to a plastic support.

Variations and modifications which will be obvious to those skilled in the art can be made in this invention without departing from the scope thereof.

I claim:

1. Diazotype phototyping material, comprising in a light sensitive layer, a light sensitive diazo component, and as a coupling component, a crystalline tetrameric condensation product of a m-polyhydric phenol with an equimolecular

amount of an aldehyde having the formula RCHO, wherein R is a hydrocarbon radical having 1-6 carbon atoms.

2. Diazotype phototyping material, comprising a plastic base impregnated with a light sensitive diazo component and with a coupling component which is a crystalline tetrameric condensation product of a m-polyhydric phenol with an equimolecular amount of an aldehyde having the formula RCHO, wherein R is a hydrocarbon radical having 1-6 carbon atoms.

3. Diazotype phototyping material, comprising in a light sensitive layer, a light sensitive diazotized p-diamine of the benzene series, and as a coupling component, a crystalline tetrameric condensation product of resorcinol with an equimolecular amount of acetaldehyde.

4. Diazotype phototyping material, comprising a paper base impregnated with the crystalline tetrameric condensation product of resorcinol with an equimolecular amount of acetaldehyde, and with the zinc chloride double salt of p-diethylaminobenzene diazonium chloride.

5. Diazotype phototyping material, comprising a plastic layer impregnated with the crystalline tetrameric condensation product of resorcinol with an equimolecular amount of acetaldehyde, and with the zinc chloride double salt of p - diethylamino - 2 - methyl benzene diazonium chloride.

6. A process for the manufacture of light sensitive diazotype materials, which comprises impregnating an absorbent base with an alcoholic solution of the crystalline tetrameric condensation product of resorcinol with an equimolecular amount of acetaldehyde, drying the base, and impregnating the latter with an aqueous solution containing the zinc chloride double salt of p-diethylaminobenzene diazonium chloride.

7. A process for the manufacture of light sensitive diazotype materials, which comprises impregnating a plastic base with an aqueous alcoholic solution containing  $\gamma$ -valerolactone, of the crystalline tetrameric condensation product of resorcinol with an equimolecular amount of acetaldehyde, and containing the zinc chloride double salt of p-diethylamino-2-methyl benzene diazonium chloride.

SAUL R. BUC.

#### REFERENCES CITED

The following references are of record in the file of this patent:

#### FOREIGN PATENTS

| Number  | Country       | Date          |
|---------|---------------|---------------|
| 491,095 | Great Britain | Aug. 26, 1938 |